

H. P. WILLIS.  
ASPHALTIC PAVEMENT AND FOUNDATION FOR PAVEMENTS.  
APPLICATION FILED JULY 10, 1916.  
**1,328,310.** Patented Jan. 20, 1920.

FIG. 1.

|                                     |
|-------------------------------------|
| { 80 to 90 % Finely-divided filler  |
| 10 to 20 % Mineral asphaltic binder |
| 1/4 to 1 % Sulfate of copper        |
| { 80 to 90 % Finely-divided filler  |
| 10 to 20 % Mineral asphaltic binder |
| 1/4 to 1 % Sulfate of copper        |

FIG. 2.

*INVENTOR.*  
*Harry Parsons Willis.*  
*BY*  
*Walter Allen.*  
*ATTORNEY.*

# UNITED STATES PATENT OFFICE.

HARRY PARSONS WILLIS, OF WATERFORD, NEW YORK, ASSIGNOR TO WILLITE ROAD CONSTRUCTION COMPANY OF AMERICA, OF NEW YORK, N. Y., A CORPORATION OF MAINE.

## ASPHALTIC PAVEMENT AND FOUNDATION FOR PAVEMENTS.

1,328,310.

Specification of Letters Patent.

Patented Jan. 20, 1920.

Original application filed December 7, 1914, Serial No. 875,767. Divided and this application filed July 10, 1916. Serial No. 108,423.

*To all whom it may concern:*

Be it known that I, HARRY PARSONS WILLIS, a citizen of the United States of America, and a resident of Waterford, in the county 5 of Saratoga and State of New York, have invented a certain new and useful Asphaltic Pavement and Foundation for Pavements, of which the following is a description, reference being had to the accompanying drawing, which forms a part of this specification.

This invention relates to pavements, especially those of asphaltic composition, but also to any pavements which are formed in layers, one or more of which comprise a 15 foundation course.

My invention comprises an asphaltic pavement made of a plurality of courses, one of which is a foundation course which can be used as a foundation for any kind of a pavement requiring a foundation, in place of the usual concrete foundation, whether the wearing course of the pavement be of bricks, asphalt, asphalt blocks, stone blocks, wooden blocks, or any kind of blocks whatsoever. 25 My invention also comprises using this foundation course with or without a wearing course of any of the above mentioned materials. Thus it may be understood that my invention comprises broadly a foundation course of a particular kind, a specific application being herein shown and described in the use of such a course in connection with an asphaltic wearing surface. In this specific application it will be noted

5 that the composition of the foundation course and the asphaltic wearing course is not precisely the same but enough alike so that the use of the one in the place of the other would still be within the scope of my invention, although not intended in actual practice, except under peculiar conditions.

This application is a divisional application of my application filed December 7, 1914, and serially numbered 875,767, allowed June 13, 1916, and patented July 11, 1916, No. 1,990,615.

My improved asphaltic pavement and foundation for pavements comprises a finely-

divided filler composed of any sand, soil, or earthy matter of any kind, or mixture thereof, of a mineral asphaltic binder and a salt having the tempering or hardening characteristics of sulfate of copper, such for instance as the sulfates or selenates of aluminium, 50 chromium, manganese, iron, indium, gallium, and sulfates or selenides of sodium, potassium, rubidium, caesium, ammonium, silver, gold, platinum or thallium, when combined with the other ingredients of the pavement, or foundation for pavements. 55

An important advantage of the invention is in the use of a filler which can be very easily and cheaply obtained, as I contemplate the use of any soil of whatsoever nature found at the place where the pavement 60 or foundation is to be made and used, or such earthy material, be it sand, disintegrated stone, clay, mixed clay, or similar material as may be obtainable at or near the place where the pavement or foundation 65 is to be placed. In the case of an old road being converted into this new pavement, the old road bed may form all or a part of the 70 filler.

This filler is finely-divided to a degree 75 such as to facilitate its incorporation, absorption or coating with the binder, but not necessarily to the degree of pulverization.

For the binder I use a mineral asphaltic material. 80

With the binder I mix a small percentage of a salt, such as sulfate of copper, or any of those above mentioned. This sets the binder and toughens it so as to increase its tensile strength and elasticity, elongation 85 and reduction of fracture. It is the use of this salt, which permeates the entire asphaltic mixture, which makes it practicable to use the cheap filler. The whole mass becomes a new chemical composition, having 90 certain characteristics, in contradistinction to all pavements and foundations known to me, which prevent its softening and flow in hot exposures, its cracking in cold exposures and eliminate its material absorption of 95 water in moist exposures, and in the case of

a foundation for a pavement, the furnishing of a particular resiliency which distributes the load over a greater area, thus reducing the possibility of the pavement breaking through vertically from sheer force, which is not attainable with the usual rigid hard concrete foundation.

In the accompanying drawing—

Figure 1 is a diagrammatic view showing 10 the composition and arrangement of an asphaltic pavement constructed according to my invention and comprising a foundation course and a wearing course.

Fig. 2 is a similar view comprising a foundation course construction according to my 15 invention and an ordinary brick or block wearing course laid on such a foundation course.

This drawing is principally for convenience in graphically illustrating the composition entering into the pavement and readily identifying the invention, therefore details 20 of construction are entirely omitted.

For the foundation or base of a pavement 25 there is taken a mixture of approximately eighty to ninety per cent. of finely-divided soil filler, generally eighty-four to ninety-two per cent. in actual practice, heated to about 350° F. To this is added from approximately 30 ten to twenty per cent. of mineral asphaltic binder, generally eight to sixteen per cent. in actual practice, also heated to about 350° F., the percentage of the binder depending on the character of the 35 filler and the quantity of the binder which the filler, heated to about the same degree, will absorb or hold as a coating. Temperatures as low as 240° have been used but it is advisable to use the higher temperature to allow 40 for losses in working. The percentage of binder in the case of sand or sand with little or no admixture of clay, for instance, is about eleven per cent. Sulfate of copper or any of the above mentioned salts, 45 from one-quarter of one per cent. to one per cent., approximately, is added to the binder during the heating of it.

Preferably the material for the filler is finely-broken or divided and heated in a 50 mixing plant. This may be in a partial vacuum and it may be mixed in a partial vacuum with the binder which has been previously heated and mixed with the sulfate of copper or any of the above mentioned salts. 55 By such process the binder permanently permeates or coats the filled thoroughly and to a degree far beyond that possible if the mixing were carried out at atmospheric pressure or without the mineral salts, and this 60 thorough permanent permeation or coating permits the use of a larger proportion of the filler than would be possible otherwise. The mixing of these materials in this manner

also insures that the product will be free from air and voids or materially denser and 65 more free from air and voids than would otherwise be the case, thus increasing the adhesion of the ingredients and the tensile strength, resiliency and toughness of the product, besides contributing to its imper- 70 meability.

For the wearing course of a pavement approximately the same materials, percentages and method of mixing may be used, but a different asphaltic material may be substituted 75 to attain a different finish.

Different degrees of smoothness and toughness and elasticity of either foundation or wearing course may be attained by varying the quantity of the filler material 80 and the proportion of sulfate of copper or the other above named salts used.

The courses are laid and rolled in the usual manner.

I have found it advisable to apply the 85 paving mixture to the road bed at a temperature approximating 350° F., for, by so doing, in the case of a multi-layer or multi-course pavement, the several layers or courses will fuse and adhere each to the 90 other, so firmly, that the structure becomes practically integral.

Though I have described with detail a specific pavement, composition and method embodying my invention, yet it is to be understood 95 that the invention is not restricted to this particular pavement, percentage and method. Various modifications thereto by those skilled in the art, with the purpose of producing a variety of 100 mechanical and ornamental finishes, through the addition of elements not affecting the chemical action of the elements of the pavement to which I lay claim, may be made 105 without departing from the spirit of my invention.

There are several advantages associated with my invention among them being the use of a universally cheap filler to the extent of approximately eighty-four to ninety-two per cent. of the total, the use of a sand, earth or mixed filler which is almost always immediately at hand, and the consequent production of a pavement at a greatly reduced expense and of a character which closely approximates perfection in lasting qualities 110 and non-injury by temperature and climatic changes. Such a pavement does not run or creep in hot weather, crack or warp in freezing weather, nor absorb any material quantity of moisture (less than  $\frac{1}{4}$  of one per cent. by test), and affords both an abundant support for very heavy loads while still possessing the resiliency so desirable and necessary for animal traffic.

As a foundation for any pavement hav-

- ing a wearing surface of other material it surpasses concrete in every particular, being water and frost proof while at the same time it is produced materially cheaper. It 5 has been the custom for years to provide all characters of "permanent" pavements, with concrete foundations in order to secure them in place both vertically and horizontally. There are instances where granite 10 block stone surfaces are essential on account of the very heavy hauling. In all such cases the resiliency of the present foundation and its weatherproofness obviate the disintegrating processes through which all of the 15 concrete foundations pass to their eventual destruction thus producing the consequent irregularity and broken parts of the wearing surfaces of the granite block pavements, which are laid on concrete foundations. 20 In the claims hereto annexed I have specified sulfate of copper specifically but it is to be understood that in specifically stating sulfate of copper I have in mind all of its equivalents so that the claims are to be construed as referring to sulfate of copper or 25 its equivalents when combined as therein set forth.
- Having thus described my invention the following is what I claim as new therein 30 and desire to secure by Letters Patent:
1. A road pavement having compression and tensile values relatively proportioned to provide characteristics of stability, resiliency and elasticity operative to resist 35 deterioration of the foundation course of the pavement in the presence of traffic load strains thereon by distributing such strains laterally of the direction of strain application, and by maintaining such characteristics in the presence of weather conditions, 40 said pavement having a foundation course consisting of a filler including finely divided earthy material of any kind, a mineral asphaltic binder and a mineral salt mixed 45 with the binder and having the characteristic of tempering the binder, said filler, binder and tempering agent being admixed in the presence of heat to produce a mixture of which the filler constitutes approximately 50 80% of the mass, the said mass when compacted producing a substantially voidless homogeneous course having the said characteristics of stability, resiliency and elasticity. 55 2. A road pavement comprising a foundation course consisting of a closely compacted mixture including finely divided earthy filler material, a mineral asphaltic binder and a mineral salt having toughening or 60 tempering properties mixed with the binder, the said filler material constituting not less than 80% of the mixture, and the amount of the tempering salt relative to the other
- components of the mixture being so proportioned as to set and toughen the binder and 65 impart to said foundation course when compacted, the properties of resiliency, tenacity and stability, whereby traffic load strains will be laterally distributed over a substantial area, thus reducing the tendency of 70 the foundation to break through vertically under such load strains. 75
3. A pavement comprising a plurality of courses, one of which is the foundation course, and said courses each being composed of a composition consisting of a finely divided filler, a mineral asphaltic binder and a mineral salt having toughening properties, 80 said courses being separately laid and compacted while the composition of one course is in a sufficiently highly heated condition whereby the courses will become intimately united by fusion to provide a practically integral structure. 85
4. A road pavement comprising a foundation course consisting of a mixture of finely divided earthy material, a mineral asphaltic binder, and a metallic salt having toughening properties, the earthy material constituting not less than 80% of the mixture, the 90 said mixture being compacted to form a foundation course substantially free from voids and characterized in this,—that it has a peculiar resiliency which operates to distribute traffic loads over a substantial 95 area, thus reducing the tendency of the foundation to break through vertically under such loads, and a wearing course overlying and fused to said foundation course, 100 said wearing course consisting of a mixture of earthy material, a mineral asphaltic binder and a metallic salt having toughening and tempering properties, the two courses being united to form a substantially integral structure. 105
5. A road pavement, comprising a foundation course consisting of a mixture composed of a filler including finely divided earthy material of any kind, a mineral asphaltic binder and a toughening or tempering mineral salt, the filler constituting approximately 80% of the mixture, the said mixture being spread and compacted directly upon mother earth to form a foundation course substantially free from voids 110 and characterized in this,—that it is sturdy, yet sufficiently resilient to distribute traffic loads over a substantial area, thus resisting the tendency of the foundation to disintegrate or break through vertically under 115 such loads, and a wearing course overlying said foundation course. 120
6. A road pavement, embodying a foundation course laid on mother earth, consisting of a mixture composed of a filler including finely divided, but not dust-like, earthy ma- 125

terial of any kind, a mineral asphaltic binder, and a mineral salt having toughening or tempering properties, the said binder constituting not less than 8% or more than 5 17% of the total mixture, and the said mixture being compacted to form a foundation course substantially free from voids and

characterized in this,—that it is sturdy, yet sufficiently resilient to distribute traffic loads over a substantial area, thus resisting 10 the tendency of the foundation to break through vertically or disintegrate under such loads.

HARRY PARSONS WILLIS.